

July 5, 1949.

K. G. RIES ET AL

**2,475,517**

## ABRASIVE ARTICLE OF MANUFACTURE

Filed Aug. 13, 1946

Fig. 1. A technical cross-sectional drawing of a composite structure. The top and bottom layers are represented by hatched rectangles. Between them are several layers: a top layer with five circular holes (9), a layer with rectangular notches (10), a layer with diagonal hatching (6), a layer with horizontal hatching (8), a central vertical column (5) with diagonal hatching, a layer with diagonal hatching (7), a layer with horizontal hatching (14), and a bottom layer with rectangular notches (15). The bottom layer also features five circular holes (12) on the left and five circular holes (13) on the right. The labels are handwritten in black ink.

Fig. 2.

Diagram of a circular component with a central hole. The component is divided into two sectors, each containing a hatched pattern. The top sector is labeled '14' and the bottom sector is labeled '7'. Two arrows, each labeled '3', point towards the top and bottom edges of the circle, indicating a rotational motion.

## UNITED STATES PATENT OFFICE

2,475,517

## ABRASIVE ARTICLE OF MANUFACTURE

Kernell G. Ries, George J. Goepfert, and George J. Easter, Niagara Falls, N. Y., assignors to The Carborundum Company, Niagara Falls, N. Y., a corporation of Delaware

Application August 13, 1946, Serial No. 690,180

4 Claims. (Cl. 51—206)

1

This invention relates to abrasive articles of manufacture and to methods of making the same. More particularly, it relates to abrasive grinding wheels of the type which comprise a resinoid bonded abrasive annulus or rim bonded to the periphery of a non-abrasive supporting center.

The invention is especially adapted to the making of diamond abrasive cutting off wheels of the aforesaid described structural type which are relatively thin, the resinoid bonded diamond annulus and the non-abrasive supporting center of the wheel usually having an overall thickness no greater than  $\frac{1}{2}$  to  $\frac{1}{8}$  of an inch and often less. The invention will therefore be primarily described as it pertains to the making of such thin diamond cutting off wheels, although it is to be understood that it is similarly applicable to the manufacture of abrasive wheels of like construction embodying other abrasive materials such as silicon carbide, fused aluminum oxide, boron carbide, and other hard granular substances of abrading or cutting ability.

It has been common practice heretofore to make abrasive wheels of the herein-described type with the non-abrasive center of molded resinoid composition. Abrasive wheels with molded resinoid centers made of the thinness necessary to render them satisfactory for cutting off purposes have been subject to frequent failure because of insufficient strength of the molded center. Efforts to meet this deficiency in strength by the provision of layers of paper or organic cloth materials as reinforcement for the molded resinoid supporting centers have been but partially satisfactory. Although such centers have shown some degree of increase in strength, they have had a marked tendency to become warped or distorted during manufacture so that the resulting abrasive wheels have not run true and have not only provided a wasteful cut but have been uneven often to the extent of absolute failure. It is also essential in a satisfactory wheel that the non-abrasive center of the wheel closely approximate in thermal coefficient of expansion that of the bonded abrasive annulus or rim. Furthermore, the shrinkage of the supporting center during the curing of the wheel should match the shrinkage of the abrasive rim in order to provide a high strength of union of the two and a resulting sound structure. Complete satisfaction in all the above respects has not been obtained by the abrasive wheel constructions provided by the prior art.

It is an object of the present invention to provide thin abrasive cutting off wheels comprising

10 a resinoid bonded abrasive rim or annulus and a non-abrasive supporting center of greater strength and durability, and having improved cutting characteristics. A further object is to provide thin abrasive wheels of the described type which, in manufacture or use, do not become warped or distorted. A still further object is the provision of an abrasive wheel of the described type in which the thermal coefficient of expansion and the shrinkage characteristics of the non-abrasive supporting center will be of the same order of magnitude as the thermal coefficient of expansion and shrinkage characteristics of the abrasive annulus. Other objects and advantages accruing from practice of the present invention will become apparent as the description proceeds.

20 In accordance with the present invention, we have found that an improved abrasive cutting-off wheel comprising an abrasive rim or annulus secured to a non-abrasive supporting center is obtained when the non-abrasive supporting center of the wheel comprises a laminated structure in which one or more of the laminations of the 25 supporting center is composed of glass fibers such as fiber glass cloth, the laminations of the supporting center being compacted and held together by impregnation with the proper amount of a resinoid binder. Such wheels have been found to be not only of increased strength but also, 30 by the control of the amount of resin in respect to the glass fiber laminations, the shrinkage characteristics and also the thermal coefficient of expansion can be controlled so as to approximate 35 the same characteristics in the bonded abrasive annulus, thereby providing increased strength and durability to the resulting article. We have further found that abrasive wheels of the described type having a supporting center comprising 40 one or more laminations of glass fibers can be additionally improved greatly in stability to warpage or distortion during manufacture and use by the inclusion of one or more laminations of wire screen in the laminated structure of the center. The fiber glass cloth, due to its inorganic 45 nature, is believed to serve the function of reducing the thermal expansion and shrinkage of the laminated center to the point where it approaches the thermal expansion and shrinkage characteristics of the abrasive annulus, provided always that the amount of impregnating resin is maintained low enough not to offset this advantage. The presence of glass fibers in the supporting 50 center serves the additional advantage of providing a structure having a low water and moisture

vapor sensitivity, which feature is particularly valuable in cutting off wheels since many cutting off operations are performed on machines designed for wet grinding. Most satisfactory results have been obtained when using woven glass cloth in making abrasive wheels of the present type when the various laminations of glass cloth are so disposed as to have the warp threads of each lamination disposed in the same direction as the warp threads of the remaining laminations of woven glass cloth.

In order that the invention may be better understood, reference is made to the accompanying drawing which is presented for illustrative purposes, and in which

Figure 1 is a vertical sectional diagrammatic view of a molding set-up adapted for making abrasive wheels in accordance with the present invention, and showing the mold set-up as it is charged preparatory to compacting and forming the abrasive wheel structure;

Figure 2 is a plan view of an abrasive wheel made in accordance with the present invention; and

Figure 3 is a vertical sectional view taken on the line 3-3 of Figure 2. The thickness of the wheel structure as shown in Figures 1 and 3 is shown in highly exaggerated form for the purpose of more clearly bringing out the actual construction of the article.

In the making of thin abrasive cutting off wheels having a non-abrasive supporting center and a peripherally bonded abrasive rim structure of the herein-described type, it is first necessary to obtain or prepare the individual resin-filled sheet material which is to go into the laminated center structure. These plies of sheet material

has been found that charging of the glass fiber cloth with a heat-hardenable resin amounting to from 40-60% by weight of the glass cloth provides shrinkage characteristics and a thermal coefficient of expansion of the material which are of the same order of magnitude as the shrinkage characteristics and thermal coefficient of expansion of resinoid bonded abrasive bodies of the type used in making abrasive wheels with which the present invention is concerned. The determination of the amount of resin to be used in any specific wheel structure will be dependent upon the shrinkage and thermal expansion characteristics of the resin bonded abrasive annulus, and will be one comparable thereto in those properties. For example, a resinoid filled laminate comprising several laminations of glass fiber cloth containing 47.3% by weight of phenol formaldehyde resin has a thermal coefficient of expansion from 26° C. to 100° C. of  $18.47 \times 10^{-6}/^{\circ}\text{C}$ . and a curing shrinkage in inches per inch of .0024. These figures compare favorably with a thermal coefficient of expansion between 26° C. and 100° C. of  $18.22 \times 10^{-6}/^{\circ}\text{C}$ . and a curing shrinkage in inches per inch of .0017 for a resin bonded abrasive body of the type used in Example I below. The thermal coefficients of expansion and curing shrinkage in inches per inch are given in Table I below for glass fiber cloth filled with different percentages by weight of a heat-hardenable phenol formaldehyde condensation product. Also shown for purposes of comparison therewith is the thermal coefficient of expansion and the shrinkage characteristics for an ordinary cotton cloth filled with 50% by weight of the same resin, showing the much greater expansion and shrinkage properties of such material.

Table I

| Type of Base Fabric            | Per Cent by Weight of Impregnating Resin | Thermal Coefficient of expansion 26° C. to 100° C. | Curing shrinkage inches/inch | Remarks                                                                                                               |
|--------------------------------|------------------------------------------|----------------------------------------------------|------------------------------|-----------------------------------------------------------------------------------------------------------------------|
| 1 Woven glass fiber cloth,     | 42.0                                     | $14.39 \times 10^{-6}/^{\circ}\text{C}$            | 0.0018                       | Low thermal coefficient of Expansion and curing shrinkage. Satisfactory for use with resin bonded abrasive bodies.    |
| 2 Do -----                     | 46.5                                     | $17.94 \times 10^{-6}/^{\circ}\text{C}$            | 0.0022                       | Do.                                                                                                                   |
| 3 Do -----                     | 54.0                                     | $19.60 \times 10^{-6}/^{\circ}\text{C}$            | 0.0022                       | Do.                                                                                                                   |
| 4 Ordinary cotton fiber cloth. | 50                                       | $20.27 \times 10^{-6}/^{\circ}\text{C}$            | 0.0050                       | High thermal coefficient of Expansion and curing shrinkage. Unsatisfactory for use with resin bonded abrasive bodies. |

are prepared by filling the layers of glass fibers such as glass cloth with an uncured resinoid binder such as phenol formaldehyde condensation product resins as, for example, that known and sold by the Bakelite Corporation under the designation "Bakelite No. BR2428".

The resin can be prepared for filling and applied in the following manner: 30 parts by weight of powdered "Bakelite" resin No. BR2428 is dissolved in a solvent mixture consisting of 40 parts by weight of acetone and 20 parts by weight of ethyl alcohol. The resulting resin solution is then applied to the glass cloth by any of the well-known ways such as dipping, spraying, brushing, or the like, and the solvents removed by heating at 150° F. for 1/2 hour.

The preparation of the above sheet material requires a control of the resin to fiber weight ratio in order that the amount of resin will not be sufficient to increase the thermal coefficient of expansion and the shrinkage characteristics of the resin-filled material to such an extent that they will be appreciably higher than those characteristics are for the particular bonded abrasive annulus of the abrasive article in which the resin-loaded materials are to be embodied. It

50 As previously stated we have found that abrasive wheels embodying a laminated center comprising one or more layers of glass fibers can be improved greatly in stability against warpage or distortion by the inclusion in the laminated center of one or more plies of wire screen. A wire screen material which has been found satisfactory for that purpose is 65 x 65 mesh size stainless steel wire screen, which is usually given a light sizing of a resin such as the resins used to 55 fill the glass fiber laminations prior to its incorporation in the laminated center. 40 x 40 mesh size tinned wire screen has also been used with satisfactory results.

60 After the preliminary preparation of the individual resin-filled laminations of fiber glass cloth as previously described, the abrasive wheels are made in the following manner. Referring to Figure 1, a mold set-up comprising a disc-shaped base plate 4 is provided with a central arbor pin 5 and an annular mold ring 6 which closely fits over the periphery of the base plate 4. The annular mold ring 6 is held in the proper position by means of shims 15 placed at suitable intervals beneath the mold ring. The resin filled 65 sheets of glass cloth 7 and the layer or layers of

## 5

resin sized wire screen 8 are cut or died out to the desired size and shape, assembled in the desired order, and placed over the arbor pin 5 so as to rest on the base plate 4. In the example shown in Figure 1, these laminations comprise two layers of resin impregnated glass cloth 7 and one intermediate layer of wire screen 8. The top mold plunger is divided into an inner arbored disc 9 having a diameter approximately the same as the non-abrasive laminated supporting center of the wheel and an outer annular ring 10 fitting around the inner disc plunger 9 and having an outside diameter equal to the diameter of the wheel to be made. The outer annular ring 10 is usually slightly thicker, e. g., .001 to .002", than the inner top plunger 9 and the base plate 4 is depressed on equal amount about the periphery so that the abrasive bonded rim when compacted will be a few thousandths of an inch thicker than the supporting center structure. After the laminations for the center structure have been placed in the mold the top plunger disc 9 is placed over the arbor pin 5 on top of the laminations to hold them compressed together. The space between the thusly positioned laminations of the supporting center and the annular mold ring 6 is then filled with the desired abrasive mixture 14 of granular abrasive material and resinoid binder. The annular ring 10 of the top mold plunger is then placed in position and the entire assembly placed between top and bottom platens 11 and 12 of a hot press, the press being heated by steam passed through conduits 13 in the press platens. The mold contents are subjected to heat and pressure to simultaneously compact and unite the individual layers of the laminated central structure, compact the annular abrasive rim, and securely bond the thusly compacted rim to the compressed supporting center. The thusly molded abrasive wheel is given a further oven cure to finally mature the resinoid binder.

While the abrasive wheels have been described above as being made by forming the laminated supporting center simultaneously with the molding and securing thereto of the bonded abrasive annulus, it is not essential that this exact procedure be followed. The laminated center can be preformed as a separate step with the abrasive rim subsequently molded and secured to the periphery of the preformed center without departing from the scope of the present invention.

In order that the present invention may be further explained, the following specific examples are given:

*Example I*

A diamond abrasive cutting off wheel 3" in diameter with a  $\frac{1}{2}$ " arbor and having a thickness of  $\frac{1}{2}$  of an inch was made as follows: Fiber glass cloth of the type designated as "Fibreglas" cloth ESS-12-261 having a thread count of 14 x 20 was secured from The Spaulding Fibre Co. of Buffalo, N. Y., filled with an uncured resin of the phenol formaldehyde type, said resin being present to the extent of 47.3% by weight of the total weight of the resin filled cloth. This resin filled fibre glass cloth was .033 inch thick. Bolting grade 65 x 65 mesh stainless mesh wire screen sold by the Buffalo Wire Company of Buffalo, N. Y., and lightly sized with a phenolic resin similar to that used for filling the glass cloth was used in the laminate. Two disc-shaped pieces of resin filled fibre glass cloth as described above and one disc-shaped piece of stainless steel wire

cloth were cut with a  $\frac{1}{2}$ " arbor hole and a diameter of approximately  $2\frac{1}{2}$ ". These disc-shaped pieces were assembled with the wire screen disposed between the two layers of resin filled glass cloth and placed in a mold such as shown in Figure 1 in the manner previously described. An abrasive mixture consisting of

|    | Parts by weight                                                                                                 |
|----|-----------------------------------------------------------------------------------------------------------------|
| 10 | 100 mesh size diamond port                                                                                      |
|    | 50                                                                                                              |
|    | Liquid phenolic resin (sold by The Bakelite Corporation under the designation "Bakelite No. XR7534")            |
|    | 3                                                                                                               |
| 15 | Powdered phenolic aldehyde resin (sold by The Bakelite Corporation under the designation "Bakelite No. BR2428") |
|    | 22                                                                                                              |
|    | Powdered cryolite filler                                                                                        |
|    | 25                                                                                                              |

was then placed in the mold space between the annular mold ring and the assembled laminations, the annular ring plunger of the mold placed in position, and the entire assembly placed in a hot press and subjected to 2000 pounds per square inch pressure and 300° F. for 30 minutes. The molded article was then cooled in the press under pressure for 5 to 10 minutes after which the molded wheel was removed from the mold and subjected to an oven cure of 16 hours at 300° F.

*Example II*

30 A diamond abrasive cutting off wheel 3" in diameter with  $\frac{1}{2}$ " arbor and  $\frac{1}{2}$ " thickness was made in accordance with the procedure set forth for Example I except for the fact that the wire screen was omitted from the laminated supporting center.

35 While we have found that thin abrasive cutting off wheels of small size comprising a resinoid bonded abrasive annulus or rim secured to a non-abrasive center embodying one or more laminations of glass fiber as the center support are improved in performance and durability over abrasive wheels of the prior art employing other types of center structures, such wheels are limited in respect to the size of wheel which can be made without warping or distortion. For that reason most satisfactory results have been obtained by the inclusion of one or more layers of wire screen in the central supporting structure in order to minimize or eliminate the warping tendency which becomes greater as the diameter size of the wheel increases. The presence or the wire screen further improves the wheel by additionally strengthening it against breakage during use. The wire screen also aids in securing the abrasive annulus to the central support by reason of the projection of the ends of the wire strands of the layer or layers of screen a slight distance into the molded abrasive annulus.

40 The tremendous improvement in the performance of abrasive wheels of the present invention embodying centers comprising laminations of glass fibers and wire screen over wheels of the prior art using molded resinoid or steel centers, is clearly demonstrated by the difference in length of service which the wheels of the present invention have given when used in the cutting off of ceramic bonded aluminum oxide resistor material. Table II below is presented to show the actual performance of thin abrasive cutting off wheels having a thickness of .032 inch as compared to the performance of similar abrasive wheels using molded resinoid centers or steel centers in the cutting off of  $\frac{1}{8}$  inch diameter rods of a very hard ceramic resistor material. The operation was conducted wet using water as the cool-

7  
ant with a wheel operating speed of 12,000  
R. P. M.

8  
ter amounting to 40% to 60% by weight of the  
resin-filled glass fabric of said center, said sup-

Table II

| Wheel<br>No. | Wheel<br>Thick-<br>ness | Type of Supporting Center                            | Abrasive Annulus                                       | No. of<br>Resis-<br>tors<br>Cut | Comparison of Percentage of Pieces Cut                                        |  |
|--------------|-------------------------|------------------------------------------------------|--------------------------------------------------------|---------------------------------|-------------------------------------------------------------------------------|--|
|              |                         |                                                      |                                                        |                                 | No. of<br>Pieces cut by Improved Wheel<br>No. of Pieces Cut by Standard Wheel |  |
| 1-----       | 1/32                    | Molded Resin.....                                    | Resinoid Bonded Diamond<br>Abrasive Composition No. 1. | 3,400                           | 100% (Standard Wheel).                                                        |  |
| 2-----       | 1/32                    | Steel.....                                           | Resinoid Bonded Abrasive Mix<br>Composition No. 2.     | 6,500                           | 190%.                                                                         |  |
| 3-----       | 1/32                    | Laminations of Fiber Glass<br>Cloth and Wire Screen. | Same as Wheel No. 1.....                               | 19,750                          | 580%.                                                                         |  |
| 4-----       | 1/32                    | Laminations of Fiber Glass<br>Cloth and Wire Screen. | Same as Wheel No. 2.....                               | 26,300                          | 775%.                                                                         |  |

Having described the invention in detail, it is  
desired to claim:

1. An abrasive cutting off wheel comprising an  
annular resinoid-bonded abrasive rim secured to  
the outer periphery of a central supporting plate  
of resin-filled, laminated fibrous structure, the  
fibrous laminations thereof comprising at least  
one layer of fibrous glass fabric and at least one  
layer of wire screen, the resin content of the non-  
abrasive center amounting to 40% to 60% by  
weight of the resin-filled glass fabric of said cen-  
ter, said supporting center having a thermal co-  
efficient of expansion between normal room tem-  
perature and 100° C. from about  $14 \times 10^{-6}/^{\circ}$  C. to about  
 $20 \times 10^{-6}/^{\circ}$  C. and a curing shrinkage in the  
neighborhood of .002" per inch, said wheel being  
substantially flat and free from distortion and  
having an overall thickness less than  $\frac{1}{16}$  of an  
inch.

2. An abrasive cutting off wheel comprising an  
annular resinoid-bonded diamond-containing  
rim secured to the outer periphery of a central  
supporting plate of resin-filled laminated fibrous  
structure, the fibrous laminations thereof com-  
prising at least one layer of fibrous glass fabric  
and at least one layer of wire screen, the resin  
content of the nonabrasive center amounting to  
40% to 60% by weight of the resin-filled glass  
fabric of said center, said supporting center hav-  
ing a thermal coefficient of expansion between  
normal room temperature and 100° C. from about  
 $14 \times 10^{-6}/^{\circ}$  C. to about  $20 \times 10^{-6}/^{\circ}$  C. and a curing  
shrinkage in the neighborhood of .002" per inch,  
said wheel being substantially flat and free from  
distortion and having an overall thickness less  
than  $\frac{1}{16}$  of an inch.

3. An abrasive cutting off wheel comprising an  
annular resinoid-bonded abrasive rim secured to  
the outer periphery of a central supporting plate  
of resin-filled laminated fibrous structure, the  
fibrous laminations thereof comprising a layer of  
wire screen between two layers of fibrous glass  
fabric, the resin content of the non-abrasive cen-

porting center having a thermal coefficient of ex-  
pansion between normal room temperature and  
100° C. from about  $14 \times 10^{-6}/^{\circ}$  C. to about  
 $20 \times 10^{-6}/^{\circ}$  C. and a curing shrinkage in the  
neighborhood of .002" per inch, said wheel being  
substantially flat and free from distortion and  
having an overall thickness less than  $\frac{1}{16}$  of an  
inch.

25 4. An abrasive cutting off wheel comprising an  
annular resinoid-bonded diamond-containing  
rim secured to the outer periphery of a central  
supporting plate of resin-filled laminated fibrous  
structure, the fibrous laminations thereof com-  
prising a layer of wire screen between two layers  
30 of fibrous glass fabric, the resin content of the  
non-abrasive center amounting to 40% to 60%  
by weight of the resin-filled glass fabric of said  
center, said supporting center having a thermal  
35 coefficient of expansion between normal room  
temperature and 100° C. from about  $14 \times 10^{-6}/^{\circ}$  C.  
to about  $20 \times 10^{-6}/^{\circ}$  C. and a curing shrinkage  
in the neighborhood of .002" per inch, said wheel  
40 being substantially flat and free from distortion  
and having an overall thickness less than  $\frac{1}{16}$  of  
an inch.

KERNELL G. RIES.  
GEORGE J. GOEPFERT.  
GEORGE J. EASTER.

## 45 REFERENCES CITED

The following references are of record in the  
file of this patent:

## 50 UNITED STATES PATENTS

| Number    | Name        | Date          |
|-----------|-------------|---------------|
| 1,977,952 | Offenbacher | Oct. 23, 1934 |
| 2,069,116 | Sanford     | Jan. 26, 1937 |
| 2,138,882 | Robie       | Dec. 6, 1938  |

## 55 FOREIGN PATENTS

| Number  | Country       | Date         |
|---------|---------------|--------------|
| 522,040 | Great Britain | June 6, 1940 |